



US005348850A

**United States Patent** [19]**Yoshida**[11] **Patent Number:** **5,348,850**[45] **Date of Patent:** **Sep. 20, 1994**[54] **SILVER HALIDE PHOTOGRAPHIC MATERIAL AND METHOD OF PROCESSING THE SAME**[75] Inventor: **Tetsuo Yoshida**, Kanagawa, Japan[73] Assignee: **Fuji Photo Film Co., Ltd.**, Kanagawa, Japan[21] Appl. No.: **112,342**[22] Filed: **Aug. 27, 1993**[30] **Foreign Application Priority Data**

Aug. 27, 1992 [JP] Japan ..... 4-228745

[51] **Int. Cl.<sup>5</sup>** ..... **G03C 1/12; G03C 1/09**[52] **U.S. Cl.** ..... **430/575; 430/427; 430/573; 430/577; 430/578; 430/579; 430/600; 430/601; 430/603; 430/610; 430/608; 430/963**[58] **Field of Search** ..... **430/575, 579, 573, 578, 430/577, 585, 600, 603, 608, 601, 610, 963, 427**[56] **References Cited****U.S. PATENT DOCUMENTS**

|           |        |                |       |         |
|-----------|--------|----------------|-------|---------|
| 4,857,450 | 8/1989 | Burrows et al. | ..... | 430/604 |
| 5,112,731 | 5/1992 | Miyasaka       | ..... | 430/567 |
| 5,215,880 | 6/1993 | Kojima et al.  | ..... | 430/603 |
| 5,238,807 | 8/1993 | Sasaki et al.  | ..... | 430/600 |

**FOREIGN PATENT DOCUMENTS**

359637 3/1991 Japan .

*Primary Examiner*—Thorl Chea*Attorney, Agent, or Firm*—Sughrue, Mion, Zinn, Macpeak & Seas[57] **ABSTRACT**

A silver halide photographic material has on a support at least one light-sensitive silver halide emulsion layer

which comprises silver halide emulsion grains having a chloride content: of at least 50 mol % and containing a metal selected from rhodium, ruthenium and rhenium in an amount of at least  $10^{-8}$  mole per mole of silver, said silver halide emulsion being spectrally sensitized with a compound of general formula (I) and being chemically sensitized with a selenium or tellurium compound:



wherein Z and Z<sub>1</sub> each represents a group of nonmetallic atoms necessary to complete a 5- or 6-membered nitrogen-containing heterocyclic nucleus; R and R<sub>1</sub> each represents an unsubstituted or substituted alkyl group, or an unsubstituted aryl group; Q and Q<sub>1</sub> each represents a group of atoms necessary to complete a 4-thiazolidinone, 5-thiazolidinone or 4-imidazolidinone nucleus; L, L<sub>1</sub> and L<sub>2</sub> each represents an unsubstituted or substituted methine group; n<sub>1</sub> and n<sub>2</sub> each represents 0 or 1; X represents an anion; and m represents 0 or 1, wherein m=0 indicates that the dye forms an inner salt. The photographic material provides high sensitivity to He—Ne laser light and ensures high contrast in the photographic images.

16 Claims, No Drawings

**SILVER HALIDE PHOTOGRAPHIC MATERIAL  
AND METHOD OF PROCESSING THE SAME**

**FIELD OF THE INVENTION**

The present invention relates to a silver halide photographic material, more particularly to a photosensitive material which ensures high sensitivity and high contrast upon short exposure using an He—Ne laser as a light source, which enables reduction in replenishment rates of processing solutions, and which has excellent suitability for rapid processing. The present invention further relates to a method of processing said material.

**BACKGROUND OF THE INVENTION**

A scanner system has recently prevailed in the graphic arts. Various kinds of light sources have been used in practice in recording apparatuses of the type which adopt a scanner system at the formation of images. In particular, a He—Ne laser has come into wide use because it is stable and can provide a high image quality. The exposure time in the scanning exposure is very short, and ranges from  $10^{-3}$  to  $10^{-7}$  second. Therefore, it is required that photosensitive materials for scanning exposure use have high sensitivity and provide high contrast images even upon such short exposure as described above.

Further, workers in the graphic arts are strongly desirous that operations be increased in speed and efficiency, that is, that the scanning operation be speeded up and the processing time of photosensitive materials be shortened. With respect to the developer and the fixer used in the processing operation, it is desirable that the amounts of developer and fixer to be used be reduced from the viewpoints of storage and recovery cost of the wastes or environmental pollution problems, so that expectations for reduction in the replenishment rates of the developer and the fixer are on the rise.

As a photosensitive material suitable for exposure with an He—Ne light source and for rapid processing, JP-A-3-59637 (the term "JP-A" as used herein means an "unexamined published Japanese patent application") discloses a photosensitive material in which carbocyanine or rhodacyanine dyes are used as spectral sensitizers and the gelatin contents of the emulsion layers and protective layers are specified. In addition, the above reference discloses in its examples silver chlorobromide emulsions which contain iridium and rhodium and which are sensitized with gold and sulfur compounds. However, the photosensitive material cited above is low in sensitivity and is not wholly satisfactory with respect to the consistency in photographic properties achieved by continuous photographic processing performed under a reduced replenishment condition, though it is satisfactory from the viewpoints of gradation and color stain.

**SUMMARY OF THE INVENTION**

Therefore, an object of the present invention is to provide a silver halide photographic material which has high sensitivity to a He—Ne laser as a light source and which ensures high contrast in the photographic images.

Another object of the present invention is to provide a photosensitive material having consistent photographic properties even when the replenishment rates

of processing solutions are reduced, and to provide a method of processing said material.

A further object of the present invention is to provide a photosensitive material which enables rapid photographic processing, and to provide a method of processing said material.

The term "rapid photographic processing" as used herein refers to a processing in which it takes the top of a photosensitive material 15 to 60 seconds to travel from the insertion slit of an automatic developing machine to the exit of the drying part of the machine via the developing tank, the transit part, the fixing tank, the transit part, the washing tank and the drying part in succession.

The above-described objects of the present invention have been attained with a silver halide photographic material which has on a support at least one layer of a light-sensitive silver halide emulsion comprising silver halide grains having a chloride content of at least 50 mole % and containing a metal selected from rhodium, ruthenium and rhenium in an amount of at least  $10^{-8}$  mole per mole of silver, said silver halide emulsion being spectrally sensitized with a compound having a structure represented by the following general formula (I) and being chemically sensitized with a selenium or tellurium compound; and with a method of processing said material:



wherein Z and  $Z_1$  each represents a group of nonmetallic atoms necessary to complete a 5- or 6-membered nitrogen-containing heterocyclic nucleus; R and  $R_1$  each represents an unsubstituted or substituted alkyl group, or an unsubstituted aryl group; Q and  $Q_1$  each represents a group of atoms necessary to complete a 4-thiazolidinone, 5-thiazolidinone or 4-imidazolidinone nucleus; L,  $L_1$  and  $L_2$  each represents an unsubstituted or substituted methine group;  $n_1$  and  $n_2$  each represents 0 or 1; X represents an anion; and m represents 0 or 1, wherein m=0 indicates that the dye forms an inner salt.

**DETAILED DESCRIPTION OF THE INVENTION**

The silver halide emulsion used in the present invention comprises silver chlorobromide or iodochlorobromide grains having a chloride content of at least 50 mole %, preferably at least 70 mole %.

The silver halide grains used in the present invention are preferably fine grains (e.g., those having an average grain size of no greater than 0.7  $\mu\text{m}$ ), especially those having an average grain size of no greater than 0.5  $\mu\text{m}$ .

The silver halide grains used in the present invention may have any crystal shape, such as that of a cube, an octahedron, a tetradecahedron, a plate or a sphere. Also, they may be a mixture of grains having different crystal shapes. However, it is desirable for them to be cubic, tetradecahedral or tabular grains.

As for the grain size distribution, it is desirable that the emulsion be monodisperse.

The term "monodisperse emulsion" as used herein refers to a silver halide emulsion having a grain size distribution represented by a variation coefficient of 20% at most, preferably 15% at most. The term "variation coefficient (%)" is defined as the value obtained by dividing the standard deviation of the silver halide grain size distribution by the average grain size and then multiplying said quotient by 100.

Photographic emulsions used in the present invention can be prepared using methods as described, e.g., in P. Glafkides, *Chemie et Physique Photographique*, Paul Montel, Paris (1967), G. F. Duffin, *Photographic Emulsion Chemistry*, The Focal Press, London (1966), V. L. Zelikman et al, *Making and Coating Photographic Emulsion*, The Focal Press, London (1964), and so on.

Specifically, any process, including an acid process, a neutral process and an ammoniacal process, may be employed. Suitable methods for reacting a water-soluble silver salt with a water-soluble halide include, e.g., a single jet method, a double jet method, or a combination thereof.

Also, a method in which silver halide grains are produced in the presence of excess silver ion (the so-called reverse mixing method) can be employed. On the other hand, the so-called controlled double jet method, in which the pAg of the liquid phase wherein silver halide grains are to be precipitated is maintained constant, may be employed.

According to this method, a silver halide emulsion having a regular crystal shape and an almost uniform distribution of grain sizes can be obtained.

For the purpose of rendering the grain sizes uniform, it is also desirable that the grain growth be accelerated within the limits of the critical saturation degree by using a method of changing the addition speed of silver nitrate or an alkali halide depending on the speed of grain growth, as disclosed in British Patent 1,535,016, JP-B-48-36890 (the term "JP-B" as used herein means an "examined Japanese patent publication") and JP-B-52-16364, or a method of changing the concentrations of the aqueous solutions, as disclosed in U.S. Pat. No. 4,242,445 and JP-A-55-158124.

The silver halide grains may differ in halide composition between the inner part and the surface layer, that is, the grains may have a so-called core/shell type structure.

With respect to the metals rhodium, ruthenium and rhenium to be used in the present invention, these metals can be used in the form of known compounds. In particular, water soluble complex salts thereof are used to advantage. The properties of these metals change greatly depending on the ligands which constitute the complex salts together with said metals, as disclosed in JP-A-2-20852 and JP-A-2-20853. These metals are used in the present invention with the intention of increasing the contrast. As for the ligands, on the other hand, it is desirable that they include halogen atoms, water molecules and nitrosyl or thionitrosyl groups as disclosed in JP-A-2-20852. In this case, the nature of the counter ion is not critical, so that conventional counter ions such as an ammonium ion or an alkali metal ion can be used as the counter ion. Specific examples of the metal complexes which can be used in the present invention are given below.



-continued

|                        |                                                     |                                                     |
|------------------------|-----------------------------------------------------|-----------------------------------------------------|
| $[\text{RhF}_6]^{-3}$  | $[\text{Rh}(\text{NO})\text{Cl}(\text{CN})_4]^{-2}$ |                                                     |
| $[\text{ReCl}_6]^{-3}$ | $[\text{Re}(\text{NO})(\text{CN})_5]^{-2}$          | $[\text{Re}(\text{NO})\text{Cl}_5]^{-2}$            |
| $[\text{ReBr}_6]^{-3}$ | $[\text{ReCl}_5(\text{NS})]^{-2}$                   | $[\text{Re}(\text{CN})_5(\text{H}_2\text{O})]^{-2}$ |
| $[\text{RuCl}_6]^{-3}$ | $[\text{Ru}(\text{NO})(\text{CN})_5]^{-2}$          | $[\text{Ru}(\text{NO})\text{Cl}_5]^{-2}$            |
| $[\text{RuBr}_6]^{-3}$ | $[\text{RuCl}_5(\text{NS})]^{-2}$                   | $[\text{Ru}(\text{CN})_5(\text{H}_2\text{O})]^{-2}$ |

In using these metal compounds, they are dissolved in water or an appropriate solvent. To stabilize such solutions, any conventional method can be used, such as a method of adding an aqueous solution of a hydrogen halide (e.g., hydrogen chloride, hydrogen bromide, hydrogen iodide) or an alkali halide (e.g., KCl, NaCl, KBr, NaBr).

Instead of using the water-soluble salts cited above, foreign silver halide grains previously doped by these metals can be added to a system for preparing the silver halide grains and dissolved therein.

The total amount of the metal compounds added in the present invention ranges properly from  $5 \times 10^{-9}$  to  $1 \times 10^{-4}$  mole, preferably from  $1 \times 10^{-8}$  to  $1 \times 10^{-6}$  mole, and particularly preferably from  $5 \times 10^{-8}$  to  $5 \times 10^{-7}$  mole, per mole of the finally prepared silver halide.

Although they can be added properly in any stage during the preparation or before the coating of the silver halide emulsion, it is particularly desirable that the metal compounds be added in the stage of grain formation so as to be incorporated in the silver halide grains. Further, compounds containing the Group VIII elements may be used in addition to the above-described metal compounds. In particular, the combined use of two or three kinds of metal compounds, which are chosen from the present metal compounds and iridium or/and iron salts, is of advantage.

As for the selenium sensitizers, known compounds can be used in the present invention. In general, chemical sensitization can be effected by adding a selenium compound of the unstable type and/or a selenium compound of the stable type to the silver halide emulsion and stirring the resulting emulsion at a high temperature of at least 40° C. for a definite time. Suitable examples of selenium compounds of the unstable type include those disclosed in JP-B-44-15748, JP-B-43-13489, JP-A-4-109240 and JP-A-4-324855, and so on. In particular, the compounds represented by the general formulae (VIII) and (IX) in JP-A-4-324855 are used to greater advantage. Specific examples of such compounds are illustrated below:



5



6

-continued



S-19



S-20

5,348,850  
S-5  
S-6  
S-7  
S-8  
S-9  
S-10  
S-11  
S-12  
S-13  
S-14  
S-15  
S-16  
S-17  
S-18  
S-19  
S-20

Tellurium sensitizers which can be used in the present invention are compounds capable of producing silver telluride, which is presumed to function as a sensitizing nucleus, on the surface or inside of silver halide grains. The production rate of silver telluride in a silver halide emulsion can be determined by the method disclosed in 20 Japanese Patent Application No. 4-146739.

Examples of such tellurium compounds include those disclosed in U.S. Pat. Nos. 1,623,449, 3,320,069 and 3,772,031, British Patents 235,211, 1,121,496, 1,295,462 and 1,396,696, Canadian Patent 800,958 and JP-A-4-204640, JP-A-4-271341, JP-A-4-333043 and Japanese Patent Application No. 4-129787; and the compounds described, e.g., in *J. Chem. Soc. Chem. Commun.*, 635 (1980); *ibid.*, 1102 (1979); *ibid.*, 645 (1979); *J. Chem. Soc. Perkin Trans.*, 1, 2191 (1980); S. Patai (editor), *The Chemistry of Organic Selenium and Tellurium Compounds*, vol. 1 (1986) and vol. 2 (1987). In particular, the compounds represented by the general formulae (II), (III) and (IV) in Japanese Patent Application No. 4-146739 are used to great advantage. Specific examples of such compounds are illustrated below:

|      |                                                                                               |     |
|------|-----------------------------------------------------------------------------------------------|-----|
| S-12 | $(nC_4H_9)_3P=Te$                                                                             | T-1 |
| 40   | $(nC_4H_9)_2P=$                                                                               | T-2 |
| 45   | $(iC_3H_7)_2PC_4H_9(n)$<br>$\begin{array}{c} Te \\    \\ (iC_3H_7)_2PC_4H_9(n) \end{array}$   | T-3 |
| 50   | $C_2H_5P(OC_2H_5)_2$<br>$\begin{array}{c} Te \\    \\ C_2H_5P(OC_2H_5)_2 \end{array}$         | T-4 |
| 55   | $(nC_4H_9O)_3P=Te$<br>$\begin{array}{c} Te \\    \\ (nC_4H_9O)_3P=Te \end{array}$             | T-5 |
| 55   |                                                                                               | T-6 |
| 60   |                                                                                               | T-7 |
| 65   | $(C_2H_5)_2PN(C_2H_5)_2$<br>$\begin{array}{c} Te \\    \\ (C_2H_5)_2PN(C_2H_5)_2 \end{array}$ | T-8 |
| 65   | $(C_2H_5)_2PN(C_2H_5)_2$<br>$\begin{array}{c} Te \\    \\ (C_2H_5)_2PN(C_2H_5)_2 \end{array}$ | T-9 |



The respective amounts of selenium and tellurium sensitizers used in the present invention, though they depend on the conditions under which the silver halide grains are ripened chemically, are generally within the range of  $10^{-8}$  to  $10^{-2}$  mole, preferably on the order of from  $10^{-7}$  to  $10^{-3}$  mole, per mole of silver halide, respectively.

Although the present invention does not impose any particular restriction on chemical sensitization, the chemical sensitization is generally carried out under conditions such that the pH is adjusted to 5 to 8, the pAg to 6 to 11, preferably 7 to 10, and the temperature to 40° to 95° C., preferably 45° to 85° C.

It is desirable in the present invention that the above-described sensitizers be used together with precious metal sensitizers, such as gold, platinum, palladium, iridium and like metal compounds. In particular, the combined use with gold sensitizers is preferred. Suitable examples of such gold sensitizers include chloroauric acid, potassium aurichlorate, potassium aurithiocyanate, auric sulfide and so on. These gold sensitizers can

be used in an amount of about  $10^{-7}$  to about  $10^{-2}$  mole per mole of silver halide.

Also, it is desirable for the above-described sensitizers to be further combined with sulfur sensitizers. As specific examples of sulfur sensitizers which can be used, there can be given known unstable sulfur compounds,

5 such as thiosulfates (e.g., hypo), thioureas (e.g., diphenyl thiourea, triethyl thiourea, allyl thiourea), rhodanines and so on. Such sulfur sensitizers can be used in 10 an amount of about  $10^{-7}$  to about  $10^{-2}$  per mole of silver halide.

15 Now, the above-illustrated formula (I) representing the sensitizing dyes used in the present invention will be described below in detail.

15 Specific examples of the nitrogen-containing heterocyclic nucleus completed by Z or  $Z_1$  include thiazole nuclei (e.g., thiazole, 4-methylthiazole, 4-phenylthiazole, 4,5-dimethylthiazole, 4,5-diphenylthiazole), benzothiazole nuclei (e.g., benzothiazole, 5-chlorobenzothiazole, 6-chlorobenzothiazole, 5-methylbenzothiazole, 6-methylbenzothiazole, 5-bromobenzothiazole, 6-bromobenzothiazole, 5-iodobenzothiazole, 6-iodobenzothiazole, 5-phenylbenzothiazole, 5-methoxybenzothiazole, 6-methoxybenzothiazole, 5-ethoxybenzothiazole, 5-ethoxycarbonylbenzothiazole, 5-hydroxybenzothiazole, 5-carboxybenzothiazole, 5-fluorobenzothiazole, 5-dimethylaminobenzothiazole, 5-acetylaminobenzothiazole, 5-trifluoromethylbenzothiazole, 5,6-dimethylbenzothiazole, 5-hydroxy-6-methylbenzothiazole, 5,6-dimethoxybenzothiazole, tetrahydrobenzothiazole), napthothiazole nuclei (e.g., naphtho[2,1-d]thiazole, naphtho[1,2-d]thiazole, naphtho[2,3-d]thiazole, 5-methoxynaphtho[1,2-d]thiazole, 7-ethoxynaphtho[2,1-d]thiazole, 8-methoxynaphtho[2,1-d]thiazole, 5-methoxynaphtho[2,3-d]thiazole),

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 965

boxyalkyl groups (e.g., carboxymethyl, 2-carboxyethyl, 3-carboxypropyl, 4-carboxybutyl, 2-(2-carboxyethoxy)ethyl), sulfoalkyl groups (e.g., 2-sulfoethyl, 3-sulfo-propyl, 3-sulfobutyl, 4-sulfobutyl, 2-hydroxy-3-sulfopropyl, 2-(3-sulfopropoxy)ethyl, 2-acetoxy-3-sulfopropyl, 3-methoxy-2-(3'-sulfopropoxy)propyl, 2-[2'-(3-sulfopropoxy)ethoxyethyl, 2-hydroxy-3-(3'-sulfopropoxy)propyl], aralkyl groups (preferably those which contain from 1 to 5 carbon atoms in their respective alkyl moieties and a phenyl group as their respective aryl moieties, with specific examples including benzyl, phenethyl, phenylpropyl, phenylbutyl, p-tolylpropyl, p-methoxyphenethyl, p-chlorophenethyl, p-carboxybenzyl, p-sulfophenethyl, p-sulfobenzyl and the like), aryloxyalkyl groups (preferably those which contain from 1 to 5 carbon atoms in their respective alkyl moieties and a phenyl group as the aryl group of their respective aryloxy moieties, with specific examples including phenoxyethyl, phenoxypropyl, phenoxybutyl, p-methylphenoxyethyl, p-methoxyphenoxypropyl and so on), vinylmethyl group, and so on. As for the aryl group, a phenyl group is an example thereof. L, L<sub>1</sub> and L<sub>2</sub> each represents an unsubstituted methine group or a substituted methine group of the formula —C(R)—. Herein, R' represents an alkyl group (e.g., methyl, ethyl), a substituted alkyl group [e.g., an alkoxyalkyl group (e.g., 2-ethoxyethyl), a carboxyalkyl group (e.g., 2-carboxyethyl), an alkoxy carbonylalkyl group (e.g., 2-methoxycarbonylethyl), an aralkyl group (e.g., benzyl, phenethyl), an aryl group (e.g., phenyl, p-methoxyphenyl,

p-chlorophenyl, o-carboxyphenyl], and so on. Further, L and L<sub>1</sub> may combine with R and R<sub>1</sub> respectively via a methine chain to complete a nitrogen-containing heterocyclic ring. Examples of a substituent group attached to the nitrogen atom present at the 3-position of a thiazoline or imidazoline nucleus completed by Q and Q<sub>1</sub> include alkyl groups (preferably those containing 1 to 8 carbon atoms, e.g., methyl, ethyl, propyl), an allyl group, aralkyl groups (preferably those containing 1-5 carbon atoms in their respective alkyl moieties, e.g., benzyl, p-carboxyphenylmethyl), aryl groups (in which the number of carbon atoms is preferably from 6 to 9 in total, e.g., phenyl, p-carboxyphenyl), hydroxyalkyl groups (preferably those containing 1 to 5 carbon atoms in their respective alkyl moieties, e.g., 2-hydroxyethyl), carboxyalkyl groups (preferably those containing 1 to 5 carbon atoms in their respective alkyl moieties, e.g., carboxymethyl), alkoxy carbonylalkyl groups (in which it is preferable for the alkyl radical of the alkoxy moiety to contain 1 to 3 carbon atoms and for the alkyl moiety to contain 1 to 5 carbon atoms, e.g., methoxycarbonyl-ethyl), and so on.

Examples of the anion represented by X include halide ions (e.g., iodide ion, bromide ion, chloride ion), perchlorate ion, thiocyanate ion, benzenesulfonate ion, p-toluenesulfonate ion, methylsulfate ion, ethylsulfate ion and so on.

Specific examples of compounds of general formula (I) are illustrated below:



-continued



I-5



I-6



I-7



I-8



I-9



I-10



I-11

5,348,850

13

14

-continued

I-12



I-13



I-14



I-15



I-16



I-17



I-18



-continued

I-19



I-20



I-21



I-22



I-23



I-24



-continued



I-25



I-26



I-27



I-28



I-29



I-30



I-31



-continued



I-32



I-33



I-34



I-35

These sensitizing dyes may be employed individually or in combination. Combinations of sensitizing dyes are often used for the purpose of supersensitization. Materials which can exhibit a supersensitizing effect in combination with a certain sensitizing dye although they themselves do not spectrally sensitize silver halide emulsions or do not absorb light in the visible region may be incorporated into the silver halide emulsions.

Useful sensitizing dyes, supersensitizing combinations of dyes and materials exhibiting a supersensitizing effect are described, e.g., in *Research Disclosure*, vol. 176, No. 17643, item IV-J at 23 page (Dec. 1978), or the above-cited patent specifications such as JP-B-49-25500, JP-B-43-4933, JP-A-59-19032, JP-A-59-192242 and so on.

It is desirable that the optimum content of sensitizing dyes be chosen depending on the grain size and the halide composition of the silver halide emulsion to be sensitized, the method and the degree of chemical sensitization, the relation between the layer to contain said sensitizing dye and the silver halide emulsion layer, the kind of an antifogging compound used together with the sensitizing dye, and so on. The determination of the optimum amount can be made by methods well-known in the art. Usually, the sensitizing dyes are used in an amount of preferably  $10^{-7}$  to  $1 \times 10^{-2}$  mole, particularly  $10^{-6}$  to  $5 \times 10^{-3}$  mole, per mole of silver halide.

The present invention does not have any particular restriction as to various kinds of additives used in the photosensitive material. For instance, the additives described in the passages of the references cited below can be preferably used.

| Items                                                                                                             | References (corresponding passages)                                                                                                                                                                                                                                                                                                                  |
|-------------------------------------------------------------------------------------------------------------------|------------------------------------------------------------------------------------------------------------------------------------------------------------------------------------------------------------------------------------------------------------------------------------------------------------------------------------------------------|
| 1) Silver halide emulsions and their preparation methods                                                          | JP-A-2-97939 (from 12th line in right lower column at page 20 to 14th line in left lower column at page 21)<br>JP-A-2-12236 (from 19th line in right upper column at page 7 to 12th line in left lower column at page 8)<br>Silver halide solvents disclosed in JP-A-4-324855                                                                        |
| 2) Sensitizing dyes usable together with the sensitizing dyes of the present invention for spectral sensitization | JP-A-2-55349 (from 8th line in left upper column at page 7 to 8th line in right lower column at page 8)<br>JP-A-2-39042 (from 8th line in right lower column at page 7 to 5th line in right lower column at page 13)                                                                                                                                 |
| 3) Antifoggants<br>Stabilizers                                                                                    | JP-A-2-103536 (from 19th line in right lower column at page 17 to 4th line in right upper column at page 18 and from 1st to 5th line in right lower column at page 18)<br>In particular, polyhydroxybenzenes as disclosed in JP-A-2-55349, from 9th line in left upper column to 17th line in right lower column at page 11, are added to advantage. |
| 4) Dyes                                                                                                           | JP-A-2-103536 (from 1st line to 18th line in right lower column at page 17)<br>JP-A-2-39042 (from 1st line in right upper column at page 4 to 5th line in right upper column at page 6)                                                                                                                                                              |
| 5) Hydrazine nucleation agents and accelerators                                                                   | JP-A-2-12236 (from 19th line in right upper column at page 2 to 3rd line in right upper column at page 7)                                                                                                                                                                                                                                            |

-continued

| Items                                             | References (corresponding passages)                                                                                                                                                                                     |
|---------------------------------------------------|-------------------------------------------------------------------------------------------------------------------------------------------------------------------------------------------------------------------------|
| 6) Surfactants<br>Antistatic<br>agents            | JP-A-2-103536 (from 13th line in right upper column at page 9 to 10th line in left upper column at page 16)<br>JP-A-2-12236 (from 7th line in right upper column to 7th line in right lower column at page 9)           |
| 7) Compounds<br>having acidic<br>groups           | JP-A-2-18542 (from 13th line in left lower column at page 2 to 18th line in right lower column at page 4)<br>JP-A-2-103536 (from 6th line in right lower column at page 18 to 1st line in left upper column at page 19) |
| 8) Hardeners                                      | JP-A-3-55349 (from 13th line in right lower column at page 8 to 8th line in left upper column at page 11)<br>JP-A-2-103536 (from 5th line to 17th line in right upper column at page 18)                                |
| 9) Matting agents,<br>Lubricants,<br>Plasticizers | JP-A-2-103536 (from 15th line in left upper column to 15th line in right upper column at page 19)                                                                                                                       |
| 10) Polymer<br>latexes                            | JP-A-2-103536 (from 12th line to 20th line in left lower column at page 18)                                                                                                                                             |
| 11) Binders                                       | JP-A-2-103536 (from 1st line to 20th line in right lower column at page 3)                                                                                                                                              |
| 12) Developers and<br>Fixers                      | JP-A-2-103536 (from 16th line in right upper column at page 19 to 8th line in left upper column at page 21)                                                                                                             |

The invention will now be illustrated in further detail by the following examples, which, however, are not intended to limit the invention in any way.

#### EXAMPLE 1

To the Solution 1 set forth in Table 1 below, which was maintained at 38° C. and pH 4.5, the Solutions 2-a and 2-b set forth in Table 1 were simultaneously added over a 16-minute period with stirring, thereby forming the grain cores. Thereto, the Solutions 3-a and 3-b set forth in Table 1 were further added over a 16-minute period, thereby forming the grain shells. Furthermore, 0.15 g of potassium iodide was admixed therewith to complete the grain formation.

As for the metal to be contained in the Solution 2-b, the metal compounds set forth in Table 7 below were used by turns in the respective amounts set forth in Table 7. As a result thereof, five (5) kinds of solutions were prepared as the Solution 2-b.

Each of the thus obtained emulsions was washed with water in a conventional manner, specifically using a flocculation method, and then 30 g of gelatin was added thereto. Each of the resulting emulsions was adjusted to pH 5.6 and pAg 7.5, and divided into three equal parts. One part was subjected to gold-sulfur sensitization with sodium thiosulfate and chloroauric acid. Another part was subjected to gold-sulfur-selenium sensitization with sodium thiosulfate, chloroauric acid and Compound S-10 illustrated hereinbefore. Still another part was subjected to gold-sulfur-tellurium sensitization with sodium thiosulfate, chloroauric acid and Compound T-15 illustrated hereinbefore. These chemical sensitization treatments were all carried out at 60° C. so as to achieve the maximum sensitivity.

To every part were further added 4-hydroxy-6-methyl-1,3,3a,7-tetraazaindene as a stabilizer in an amount of 20 mg and phenoxyethanol as an antiseptic in an amount equivalent to 100 ppm. Thus, fifteen (15) different silver iodochlorobromide cubic grain emulsions (variation coefficient: 9%) having a chloride content of 80 mole %

and an average grain size of 0.20  $\mu\text{m}$ , which are shown in Table 7, were obtained.

TABLE 1

| Compositions of Solutions used |                                                                                                                                       |                                                               |
|--------------------------------|---------------------------------------------------------------------------------------------------------------------------------------|---------------------------------------------------------------|
| 5                              | <u>Solution 1:</u><br>Water<br>Gelatin<br>Sodium Chloride<br>1,3-Dimethylimidazolidinone-2-thione<br>Sodium Benzenethiosulfonate      | 1 l<br>20 g<br>2 g<br>20 mg<br>6 mg                           |
| 10                             | <u>Solution 2-a:</u><br>Water<br>Silver Nitrate                                                                                       | 300 ml<br>100 g                                               |
| 15                             | <u>Solution 2-b:</u><br>Water<br>Sodium Chloride<br>Potassium Bromide<br>Potassium Hexachloroiodate(III)<br>Compound shown in Table 7 | 300 ml<br>30 g<br>14 g<br>15 ml<br>amount shown<br>in Table 7 |
| 20                             | <u>Solution 3-a:</u><br>Water<br>Silver Nitrate                                                                                       | 300 ml<br>100 g                                               |
| 25                             | <u>Solution 3-b:</u><br>Water<br>Sodium Chloride<br>Potassium Bromide                                                                 | 300 ml<br>30 g<br>14 g                                        |

To each of the thus obtained emulsions, there were added 150 mg/mole Ag of Sensitizing Dye I-5 illustrated hereinbefore, 75 mg/mole Ag of disodium 4,4'-bis(4,6-naphthoxy-pyrimidin-2-ylamino)stilbenedisulfonate as a supersensitizer, 25 mg/mole Ag of 1-phenyl-5-mercaptopotetrazole as a stabilizer and 6 g/mole Ag of hydroquinone.

Further, polyethylacrylate latex and 0.01  $\mu\text{m}$  colloidal silica were each added in a proportion of 30 weight % with respect to the gelatin binder, and 2-bis(vinylsulfonylacetamide)-ethane was added at a coverage of 70 mg/m<sup>2</sup>. Then, the resulting emulsions were coated on separate polyester supports so as to have a silver coverage of 3.2 g/m<sup>2</sup> and a gelatin coverage of 1.4 g/m<sup>2</sup>. In coating each emulsion, the upper and the lower protective layers having the individual compositions shown in Table 2 below were coated simultaneously. Additionally, every support used had on the back side a BC layer and a BC protective layer having the individual compositions shown in Table 3 below.

TABLE 2

| Constitutions of Protective Layers                               |                    |
|------------------------------------------------------------------|--------------------|
| Ingredient                                                       | per m <sup>2</sup> |
| <u>Lower Protective Layer:</u>                                   |                    |
| Gelatin                                                          | 0.25 g             |
| Dye (a) illustrated below                                        | 250 mg             |
| 1,5-Dihydroxy-2-benzaldoxime                                     | 25 mg              |
| 5-Chloro-8-hydroxyquinoline                                      | 5 mg               |
| Polyethylacrylate latex                                          | 160 mg             |
| Sodium benzenethiosulfonate                                      | 5 mg               |
| $\alpha$ -Lipoic acid                                            | 5 mg               |
| Compound (b) illustrated below                                   | 5 mg               |
| Compound (c) illustrated below                                   | 100 mg             |
| Polyacrylamide<br>(average molecular weight 5,000)               | 500 mg             |
| <u>Upper Protective Layer:</u>                                   |                    |
| Gelatin                                                          | 0.25 g             |
| Silica matting agent<br>(average grain size: 2.5 $\mu\text{m}$ ) | 30 mg              |
| Silicone oil                                                     | 100 mg             |
| Colloidal silica<br>(grain diameter: 10 $\mu\text{m}$ )          | 30 mg              |
| Compound (d) illustrated below                                   | 5 mg               |

TABLE 2-continued

| Constitutions of Protective Layers |                    |
|------------------------------------|--------------------|
| Ingredient                         | per m <sup>2</sup> |
| Sodium dodecylbenzenesulfonate     | 22 mg              |
| (a)                                |                    |
| (b)                                |                    |
| (c)                                |                    |
| (d)                                |                    |

TABLE 3

TABLE 3-continued

| Constitutions of Backing Layers       |                    |
|---------------------------------------|--------------------|
| Ingredient                            | per m <sup>2</sup> |
| 5 2-Bis(vinylsulfonylacetamido)ethane | 160 mg             |
| (e)                                   |                    |
| 10                                    |                    |
| 15                                    |                    |
| 20                                    |                    |
| 25                                    |                    |
| 30                                    |                    |

## Evaluation of Photographic Properties

| Constitutions of Backing Layers                                                     |                    |
|-------------------------------------------------------------------------------------|--------------------|
| Ingredient                                                                          | per m <sup>2</sup> |
| <u>BC Layer:</u>                                                                    |                    |
| Gelatin                                                                             | 0.25 mg            |
| Sodium dodecylbenzenesulfonate                                                      | 20 mg              |
| SnO <sub>2</sub> /SbO <sub>2</sub> (9/1 by weight)<br>(average grain size: 0.25 μm) | 300 mg             |
| <u>BC Protective Layer:</u>                                                         |                    |
| Gelatin                                                                             | 2.8 g              |
| Polymethylmethacrylate                                                              | 50 mg              |
| (average particle size: 3.5 μm)                                                     |                    |
| Dye (e) illustrated below                                                           | 35 mg              |
| Dye (f) illustrated below                                                           | 35 mg              |
| Dye (g) illustrated below                                                           | 120 mg             |
| Sodium dodecylbenzenesulfonate                                                      | 90 mg              |
| Compound (d) illustrated above                                                      | 10 mg              |

The thus prepared samples each were subjected to sensitometry by being exposed with a Xenon flash light having an emission time of  $10^{-5}$  second via an interference filter having its peak at 633 nm and a continuous wedge, and then being photographically processed with an automatic developing machine, Automatic Processor FG-710S, made by Fuji Photo Film Co., Ltd., operated under the conditions described in Table 4 below. Each sample was examined for the amount of exposure required to provide a density of 3.0, and the reciprocal of said amount was taken as the sensitivity thereof. The sensitivities so determined are shown as relative values. In addition, the slope of the line connecting the points at which the densities were 0.1 and 3.0 respectively was defined as the gradient.

TABLE 4

| Processing Condition adopted in FG 710S |             |                   |
|-----------------------------------------|-------------|-------------------|
| Steps                                   | Temperature | Time              |
| Insertion                               |             | 2 seconds         |
| Development                             | 38° C.      | 16 seconds        |
| Fixation                                | 37° C.      | 16 seconds        |
| Washing                                 | 26° C.      | 9 seconds         |
| Squeeze                                 |             | 3 seconds         |
| Drying                                  | 55° C.      | <u>15 seconds</u> |
| Total processing time:                  |             | 61 seconds        |

The developer and the fixer used herein had the compositions described in Table 5 and Table 6 below, respectively.

TABLE 5

| Composition of Developer                          |         |
|---------------------------------------------------|---------|
| Sodium 1,2-dihydroxybenzene-3,5-disulfonate       | 0.5 g   |
| Diethylenetriaminetetraacetic acid                | 2.0 g   |
| Sodium carbonate                                  | 5.0 g   |
| Boric acid                                        | 10.0 g  |
| Potassium sulfite                                 | 85.0 g  |
| Sodium bromide                                    | 6.0 g   |
| Diethylene glycol                                 | 40.0 g  |
| 5-Methylbenzotriazole                             | 0.2 g   |
| Hydroquinone                                      | 30.0 g  |
| 4-Hydroxymethyl-4-methyl-1-phenyl-3-pyrazolidone  | 1.6 g   |
| 2,3,5,6,7,8-hexahydro-2-thioxo-4-(1H)-quinalizine | 0.05 g  |
| Sodium 2-mercaptopbenzimidazole-5-sulfonate       | 0.3 g   |
| Water to make                                     | 1 l     |
| Potassium hydroxide to adjust                     | pH 10.7 |

TABLE 6

| Composition of Fixer                           |          |
|------------------------------------------------|----------|
| Sodium thiosulfate (anhydrous)                 | 150 g    |
| Compound-h shown below                         | 0.1 mole |
| Sodium hydrogen sulfite                        | 30 g     |
| Disodium ethylenediaminetetraacetate dihydrate | 25 g     |
| Water to make                                  | 1 l      |
| Sodium hydroxide to adjust                     | pH 6.0   |



The results obtained are shown in Table 7 below.

TABLE 7

| Sample No. | Species of Compound                   | Amount added (mol/mol Ag) | Chemical Sensitization*1 | Sensitivity | Gradient | Fog  | Note       |
|------------|---------------------------------------|---------------------------|--------------------------|-------------|----------|------|------------|
| 1          | —                                     | —                         | S + Au                   | 100         | 5.0      | 0.05 | Comparison |
| 2          | —                                     | —                         | Se + S + Au              | 110         | 4.5      | 0.09 | Comparison |
| 3          | —                                     | —                         | Te + S + Au              | 105         | 4.4      | 0.12 | Comparison |
| 4          | NH <sub>3</sub> RhCl <sub>6</sub>     | 1.5 × 10 <sup>-7</sup>    | S + Au                   | 60          | 7.0      | 0.05 | Comparison |
| 5          | NH <sub>3</sub> RhCl <sub>6</sub>     | 1.5 × 10 <sup>-7</sup>    | Se + S + Au              | 88          | 7.8      | 0.05 | Invention  |
| 6          | NH <sub>3</sub> RhCl <sub>6</sub>     | 1.5 × 10 <sup>-7</sup>    | Te + S + Au              | 85          | 7.6      | 0.05 | Invention  |
| 7          | K <sub>3</sub> ReCl <sub>6</sub>      | 4 × 10 <sup>-7</sup>      | S + Au                   | 61          | 6.8      | 0.05 | Comparison |
| 8          | K <sub>3</sub> ReCl <sub>6</sub>      | 4 × 10 <sup>-7</sup>      | Se + S + Au              | 88          | 7.9      | 0.05 | Invention  |
| 9          | K <sub>3</sub> ReCl <sub>6</sub>      | 4 × 10 <sup>-7</sup>      | Te + S + Au              | 85          | 7.3      | 0.05 | Invention  |
| 10         | K <sub>2</sub> RuCl <sub>5</sub> (NO) | 2 × 10 <sup>-7</sup>      | S + Au                   | 58          | 7.0      | 0.05 | Comparison |
| 11         | K <sub>2</sub> RuCl <sub>5</sub> (NO) | 2 × 10 <sup>-7</sup>      | Se + S + Au              | 85          | 7.9      | 0.05 | Invention  |
| 12         | K <sub>2</sub> RuCl <sub>5</sub> (NO) | 2 × 10 <sup>-7</sup>      | Te + S + Au              | 83          | 7.7      | 0.05 | Invention  |
| 13         | K <sub>3</sub> Fe(CN) <sub>6</sub>    | 2 × 10 <sup>-6</sup>      | S + Au                   | 100         | 4.6      | 0.05 | Comparison |
| 14         | K <sub>3</sub> Fe(CN) <sub>6</sub>    | 2 × 10 <sup>-6</sup>      | Se + S + Au              | 105         | 4.3      | 0.05 | Comparison |
| 15         | K <sub>3</sub> Fe(CN) <sub>6</sub>    | 2 × 10 <sup>-6</sup>      | Te + S + Au              | 108         | 4.2      | 0.05 | Comparison |

\*1: S, Se, Te and Au represent sulfur sensitization, selenium sensitization, tellurium sensitization and gold sensitization respectively.

As can be seen from the data set forth in Table 7, the system free from any metal relating to the present invention and the system containing the salt of Fe as a metal for comparison caused a decrease of gradient and 5 an increase of fog by the selenium or tellurium sensitization carried out in combination with sulfur-gold sensitization, while these sensitization treatments succeeded in increasing both the sensitivity and the gradient in the samples prepared in accordance with embodiments of 10 the present invention, namely Sample Nos. 5, 6, 8, 9, 11 and 12.

### EXAMPLE 2

Similarly to the samples in Example 1, there were 15 prepared emulsions for comparison, Sample Nos. 16, 17 and 18 (which underwent different chemical sensitization treatments, S+Au, Se+S+Au and Te+S+Au, respectively). In preparing them,  $1.5 \times 10^{-7}$  mole/mole Ag of NH<sub>3</sub>RhCl<sub>6</sub> was used in the Solution 2-b as the 20 compound shown in Table 7 and the amounts of sodium chloride and potassium bromide used in both the Solutions 2-b and 3-b were changed so that the resulting emulsions might have a chloride content of 40 mole %. These samples and certain of the samples prepared in 25 Example 1 were each subjected to the same photographic processing as in Example 1, except that the development time was reduced to 12 seconds by increasing the linear speed of the automatic developing machine. The results obtained are shown in Table 8 30 below.

TABLE 8

| Sample No. | Species of Compound                   | Chloride Content (mole %) | Chemical Sensitization*1 | Sensitivity | Gradient | Fog  | Note       |
|------------|---------------------------------------|---------------------------|--------------------------|-------------|----------|------|------------|
| 4          | NH <sub>3</sub> RhCl <sub>6</sub>     | 80                        | S + Au                   | 50          | 6.6      | 0.05 | Comparison |
| 5          | NH <sub>3</sub> RhCl <sub>6</sub>     | 80                        | Se + S + Au              | 88          | 7.8      | 0.05 | Invention  |
| 6          | NH <sub>3</sub> RhCl <sub>6</sub>     | 80                        | Te + S + Au              | 85          | 7.6      | 0.05 | Invention  |
| 7          | K <sub>3</sub> ReCl <sub>6</sub>      | 80                        | S + Au                   | 51          | 6.0      | 0.05 | Comparison |
| 8          | K <sub>3</sub> ReCl <sub>6</sub>      | 80                        | Se + S + Au              | 87          | 8.0      | 0.05 | Invention  |
| 9          | K <sub>3</sub> ReCl <sub>6</sub>      | 80                        | Te + S + Au              | 84          | 7.4      | 0.05 | Invention  |
| 10         | K <sub>2</sub> RuCl <sub>5</sub> (NO) | 80                        | S + Au                   | 48          | 6.3      | 0.05 | Comparison |
| 11         | K <sub>2</sub> RuCl <sub>5</sub> (NO) | 80                        | Se + S + Au              | 85          | 7.9      | 0.05 | Invention  |
| 12         | K <sub>2</sub> RuCl <sub>5</sub> (NO) | 80                        | Te + S + Au              | 84          | 7.8      | 0.05 | Invention  |
| 13         | K <sub>3</sub> Fe(CN) <sub>6</sub>    | 80                        | S + Au                   | 80          | 4.0      | 0.05 | Comparison |
| 14         | K <sub>3</sub> Fe(CN) <sub>6</sub>    | 80                        | Se + S + Au              | 85          | 3.8      | 0.10 | Comparison |
| 15         | K <sub>3</sub> Fe(CN) <sub>6</sub>    | 80                        | Te + S + Au              | 88          | 3.6      | 0.15 | Comparison |
| 16         | NH <sub>3</sub> RhCl <sub>6</sub>     | 40                        | S + Au                   | 80          | 6.0      | 0.05 | Comparison |

TABLE 8-continued

| Sample No. | Species of Compound               | Chloride Content (mole %) | Chemical Sensitization*1 | Sensitivity | Gradient | Fog  | Note       |
|------------|-----------------------------------|---------------------------|--------------------------|-------------|----------|------|------------|
| 17         | NH <sub>3</sub> RhCl <sub>6</sub> | 40                        | Se + S + Au              | 78          | 6.8      | 0.05 | Comparison |
| 18         | NH <sub>3</sub> RhCl <sub>6</sub> | 40                        | Te + S + Au              | 75          | 6.6      | 0.05 | Comparison |

\*1: S, Se, Te and Au represent sulfur sensitization, selenium sensitization, tellurium sensitization and gold sensitization respectively.

As can be seen from Table 8, both high sensitivity and high contrast were achieved by the present samples even in case of rapid processing.

### EXAMPLE 3

Films having 3.6 g/m<sup>2</sup>, based on silver, of a coating of a silver chlorobromide emulsion having a chloride content of 70 mole % were subjected to continuous processing with an automatic developing machine, FG-710S, the same as used for the evaluation of sensitivity in the foregoing examples, under a condition such that the sample films, some of which were exposed to light and others of which were unexposed, were processed at a replenishment rate of 180 ml/m<sup>2</sup> in each mother solutions for development and fixation. A ratio of the exposed and the unexposed sample films processed, were 1:1. The processing was continued until the total area of the both processed films was brought up to 150 m<sup>2</sup>. The thus obtained processing solutions were used in evaluating the sensitivity at 633 nm and the gradient, and the evaluation result of these properties was expressed in terms of the difference between the results obtained using the fresh processing solutions and those obtained using the continuously used ones. Further, the clarity upon fixation was also evaluated.

The samples used for the evaluation were the same as used in Example 2. The results obtained are shown in Table 9 below.

were evaluated under the same conditions as in Example 2.

Further, these samples were examined for color stain, and the evaluation thereof was made in terms of five relative grades, with 5 being the best and 1 being the worst.

The results obtained are shown in Table 10 below.

TABLE 10

| Sample No. | Sensitizing Dye | Sensitivity | Gradient | Fog | Color stain | Note |
|------------|-----------------|-------------|----------|-----|-------------|------|
| 20         | 5               | I-5         | 88       | 7.6 | 0.05        | 5    |
|            | 19              | I-8         | 90       | 7.6 | 0.05        | 5    |
|            | 20              | I-7         | 92       | 7.7 | 0.05        | 5    |
|            | 21              | I-13        | 85       | 7.6 | 0.05        | 5    |
|            | 22              | (h)         | 60       | 7.4 | 0.07        | 2    |
| 25         | 23              | (I)         | 80       | 7.6 | 0.08        | 1    |
|            | 24              | (J)         | 58       | 7.5 | 0.07        | 2    |



TABLE 9

| Sample No. | Species of Compound                   | Chloride Content (mole %) | Chemical Sensitization*1 | 12 seconds' Development |                     |                       | 16 seconds' Development |                     |                       |
|------------|---------------------------------------|---------------------------|--------------------------|-------------------------|---------------------|-----------------------|-------------------------|---------------------|-----------------------|
|            |                                       |                           |                          | Change for Sensitivity  | Change for Gradient | Clarity Upon Fixation | Change for Sensitivity  | Change for Gradient | Clarity Upon Fixation |
| 4          | NH <sub>3</sub> RhCl <sub>6</sub>     | 80                        | S + Au                   | -35                     | -1.0                | good                  | -10                     | -0.6                | good                  |
| 5          | NH <sub>3</sub> RhCl <sub>6</sub>     | 80                        | Se + S + Au              | -2                      | -0.1                | good                  | 0                       | 0                   | good                  |
| 6          | NH <sub>3</sub> RhCl <sub>6</sub>     | 80                        | Te + S + Au              | 0                       | 0                   | good                  | 0                       | 0                   | good                  |
| 7          | K <sub>3</sub> ReCl <sub>6</sub>      | 80                        | S + Au                   | -35                     | -1.0                | good                  | -10                     | -0.6                | good                  |
| 8          | K <sub>3</sub> ReCl <sub>6</sub>      | 80                        | Se + S + Au              | -3                      | -0.1                | good                  | 0                       | 0                   | good                  |
| 9          | K <sub>3</sub> ReCl <sub>6</sub>      | 80                        | Te + S + Au              | -4                      | 0                   | good                  | 0                       | 0                   | good                  |
| 10         | K <sub>2</sub> RuCl <sub>5</sub> (NO) | 80                        | S + Au                   | -38                     | -1.0                | good                  | -10                     | -0.6                | good                  |
| 11         | K <sub>2</sub> RuCl <sub>5</sub> (NO) | 80                        | Se + S + Au              | -2                      | -0.1                | good                  | 0                       | 0                   | good                  |
| 12         | K <sub>2</sub> RuCl <sub>5</sub> (NO) | 80                        | Te + S + Au              | -3                      | -0.2                | good                  | 0                       | 0                   | good                  |
| 13         | K <sub>3</sub> Fe(CN) <sub>6</sub>    | 80                        | S + Au                   | -48                     | -1.0                | good                  | -10                     | -0.6                | good                  |
| 14         | K <sub>3</sub> Fe(CN) <sub>6</sub>    | 80                        | Se + S + Au              | -40                     | -0.7                | good                  | -8                      | -0.4                | good                  |
| 15         | K <sub>3</sub> Fe(CN) <sub>6</sub>    | 80                        | Te + S + Au              | -38                     | -0.8                | good                  | -9                      | -0.6                | good                  |
| 16         | NH <sub>3</sub> RhCl <sub>6</sub>     | 40                        | S + Au                   | -48                     | -1.0                | no good               | -10                     | -0.6                | good                  |
| 17         | NH <sub>3</sub> RhCl <sub>6</sub>     | 40                        | Se + S + Au              | -28                     | -0.8                | no good               | -10                     | -0.5                | good                  |
| 18         | NH <sub>3</sub> RhCl <sub>6</sub>     | 40                        | Te + S + Au              | -30                     | -0.7                | no good               | -15                     | -0.4                | good                  |

\*1: S, Se, Te and Au represent sulfur sensitization, selenium sensitization, tellurium sensitization and gold sensitization respectively.

As can be seen from Table 9, the samples of the present invention achieved consistent results in terms of their photographic properties and had good fixability in both general and rapid processing operations even when these operations were performed continuously.

### EXAMPLE 4

Samples were prepared in the same manner as Sample No. 5 prepared in Example 1, except that the Sensitizing Dye I-5 was replaced by those shown in Table 10 respectively. The photographic properties of the samples



The results in Table 10 show that the sensitizing dyes of the present invention proved to be superior in color stain to the dyes used for comparison.

While the invention has been described in detail and with reference to specific embodiments thereof, it will be apparent to one skilled in the art that various changes and modifications can be made therein without departing from the spirit and scope thereof.

What is claimed is:

1. A silver halide photographic material which has on a support at least one layer of a light-sensitive silver halide emulsion comprising silver halide grains having a chloride content of at least 50 mole % and containing a metal selected from rhodium, ruthenium and rhenium in an amount of at least  $10^{-8}$  mole per mole of silver, said silver halide emulsion being spectrally sensitized with a compound having a structure represented by the following general formula (I) and being chemically sensitized with a selenium or tellurium compound:



wherein Z and Z<sub>1</sub> each represents a group of nonmetallic atoms necessary to complete a 5- or 6-membered nitrogen-containing heterocyclic nucleus; R and R<sub>1</sub> each represents an unsubstituted or substituted alkyl group, or an unsubstituted aryl group; Q and Q<sub>1</sub> each represents a group of atoms necessary to complete a 4-thiazolidinone, 5-thiazolidinone or 4-imidazolidinone nucleus; L, L<sub>1</sub> and L<sub>2</sub> each represents an unsubstituted or substituted methine group; n<sub>1</sub> and n<sub>2</sub> each represents 0 or 1; X represents an anion; and m represents 0 or 1, wherein m=0 indicates that the dye forms an inner salt.

2. The silver halide photographic material of claim 1, wherein the silver halide grains in the silver halide emulsion have a chloride content of at least 70 mole %.

3. The silver halide photographic material of claim 1, wherein the silver halide grains in the silver halide emulsion are fine grains having an average grain size no greater than 0.7 microns.

4. The silver halide photographic material of claim 1, wherein the silver halide grains in the silver halide emulsion are fine grains having an average grain size no greater than 0.5 microns.

5. The silver halide photographic material of claim 1, wherein the silver halide grains in the silver halide emulsion are cubic, tetradecahedral, or tabular grains.

6. The silver halide photographic material of claim 1, wherein the silver halide emulsion is a monodisperse emulsion.

7. The silver halide photographic material of claim 1, wherein the metal selected from rhodium, ruthenium and rhenium is incorporated in the silver halide grains in the form of a water soluble complex salt of the metal.

8. The silver halide photographic material of claim 7, wherein the total amount of the water soluble complex salt of the metal is from  $5 \times 10^{-9}$  to  $1 \times 10^{-4}$  mol per mole of silver halide in the emulsion.

9. The silver halide photographic material of claim 7, wherein the total amount of the water soluble complex

salt of the metal is from  $1 \times 10^{-8}$  to  $1 \times 10^{-6}$  mol per mole of silver halide in the emulsion.

10. The silver halide photographic material of claim 7, wherein the total amount of the water soluble complex salt of the metal is from  $5 \times 10^{-8}$  to  $1 \times 10^{-7}$  mol per mole of silver halide in the emulsion.

11. The silver halide photographic material of claim 1, wherein the amount of the selenium or tellurium compound is from  $10^{-8}$  to  $10^{-2}$  mole per mole of silver halide in the emulsion.

12. The silver halide photographic material of claim 1, wherein the amount of the selenium or tellurium compound is from  $10^{-7}$  to  $10^{-3}$  mole per mole of silver halide in the emulsion.

13. The silver halide photographic material of claim 1, wherein the silver halide emulsion is further sensitized with a precious metal sensitizer.

14. The silver halide photographic material of claim 13, wherein the silver halide emulsion is further sensitized with a sulfur sensitizer.

15. A method of processing a silver halide photographic material which comprises image-wise exposing said photographic material and processing said photographic material with an automatic developing machine wherein the replenishment rates of a developer and a fixer are each controlled to at most  $200 \text{ ml/m}^2$ , wherein said photographic material comprises on a support at least one layer of a light-sensitive silver halide emulsion comprising silver halide grains having a chloride content of at least 50 mole % and containing a metal selected from rhodium, ruthenium and rhenium in an amount of at least  $10^{-8}$  mole per mole of silver, said silver halide emulsion being spectrally sensitized with a compound having a structure represented by the following general formula (I) and being chemically sensitized with a selenium or tellurium compound:



wherein Z and Z<sub>1</sub> each represents a group of nonmetallic atoms necessary to complete a 5- or 6-membered nitrogen-containing heterocyclic nucleus; R and R<sub>1</sub> each represents an unsubstituted or substituted alkyl group, or an unsubstituted aryl group; Q and Q<sub>1</sub> each represents a group of atoms necessary to complete a 4-thiazolidinone, 5-thiazolidinone or 4-imidazolidinone nucleus; L, L<sub>1</sub> and L<sub>2</sub> each represents an unsubstituted or substituted methine group; n<sub>1</sub> and n<sub>2</sub> each represents 0 or 1; X represents an anion, m represents 0 or 1, wherein m=0 indicates that the dye forms an inner salt.

16. A method of processing a silver halide photographic material which comprises image-wise exposing said photographic material and processing said photographic material with an automatic developing machine wherein the total processing time is adjusted so as to be within the range of 15 to 60 seconds, wherein said photographic material comprises on a support at least one layer of a light-sensitive silver halide emulsion comprising silver halide grains having a chloride content of at least 50 mole % and containing a metal selected from

rhodium, ruthenium and rhenium in an amount of at least  $10^{-8}$  mole per mole of silver, said silver halide emulsion being spectrally sensitized with a compound having a structure represented by the following general formula (I) and being chemically sensitized with a selenium or tellurium compound:



(I)

wherein Z and Z<sub>1</sub> each represents a group of nonmetallic atoms necessary to complete a 5- or 6-membered nitrogen-containing heterocyclic nucleus; R and R<sub>1</sub> each represents an unsubstituted or substituted alkyl group, or an unsubstituted aryl group; Q and Q<sub>1</sub> each represents a group of atoms necessary to complete a 4-thiazolidinone, 5-thiazolidinone or 4-imidazolidinone nucleus; L, L<sub>1</sub> and L<sub>2</sub> each represents an unsubstituted or substituted methine group; n<sub>1</sub> and n<sub>2</sub> each represents 0 or 1; X represents an anion; m represents 0 or 1, wherein m=0 indicates that the dye forms an inner salt.

-continued



wherein Z and Z<sub>1</sub> each represents a group of nonmetallic atoms necessary to complete a 5- or 6-membered nitrogen-containing heterocyclic nucleus; R and R<sub>1</sub> each represents an unsubstituted or substituted alkyl group, or an unsubstituted aryl group; Q and Q<sub>1</sub> each represents a group of atoms necessary to complete a 4-thiazolidinone, 5-thiazolidinone or 4-imidazolidinone nucleus; L, L<sub>1</sub> and L<sub>2</sub> each represents an unsubstituted or substituted methine group; n<sub>1</sub> and n<sub>2</sub> each represents 0 or 1; X represents an anion; m represents 0 or 1, wherein m=0 indicates that the dye forms an inner salt.

\* \* \* \* \*

20

25

30

35

40

45

50

55

60

65